

# UNITED STATES PATENT OFFICE.

FRANK K. CAMERON, OF WASHINGTON, DISTRICT OF COLUMBIA, AND RICHARD B. MOORE, OF INDIANAPOLIS, INDIANA.

PROCESS FOR EXTRACTING IODIN, CHLORIN, POTASSIUM HYDROXID, AND OTHER USEFUL PRODUCTS FROM THE ASH OF SEAWEEDS OR OTHER MARINE FORMS OF ALGÆ.

1,051,984.

Specification of Letters Patent. Patented Feb. 4, 1913.

No Drawing.

Application filed December 26, 1911. Serial No. 668,007.

(DEDICATED TO THE PUBLIC.)

To all whom it may concern:

Be it known that we, FRANK K. CAMERON and RICHARD B. MOORE, citizens of the United States, and employees of the Department of

5 Agriculture, said FRANK K. CAMERON residing in the city of Washington, District of Columbia, (whose post-office address is Washington, District of Columbia,) and said RICHARD B. MOORE being a legal resident of the city of Indianapolis, of the State 10 of Indiana, temporarily residing in the city of Washington, District of Columbia, (whose post-office address is Washington, District of Columbia,) have invented a new 15 and useful Process for Extracting Iodin, Chlorin, Potassium Hydroxid, and other Useful Products from the Ash of Seaweeds or other Marine Forms of *Algae*.

This application is made under the act of 20 March 3, 1883, chapter 143 (22 Stat., 625), and the invention herein described and claimed may be used by the Government of the United States or any of its officers or employees in the prosecution of work for 25 the United States, or by any person in the United States, without the payment of any royalty thereon.

The object of our invention is to provide 30 a method for extracting iodin, chlorin, potassium hydroxid and other useful products from the residue obtained by the partial or complete charring of seaweeds or other marine forms of *Algae*.

It is well known that the residue or ash of 35 seaweeds consists very largely of potassium chlorid with traces of iodids and other salts. By long experiments we have evolved a process for extracting these products from the ash. The separation may be performed 40 in two ways. According to one mode of treatment the ash is lixiviated with water and the solution filtered or drawn off from the insoluble portion by any well known method. The solution is then evaporated 45 until the less soluble salts crystallize out. After this operation, the mother liquor containing all the soluble iodids and some of the chlorids is subjected to the following treatment: The mother liquor is placed in 50 the anode compartment of an electrolytic cell. Such anode compartment is separated

from the cathode compartment by means of a diaphragm composed of any suitable material but preferably of unglazed porcelain or earthenware. On the passage of an electrolytic current the chlorin and iodin appear at the anode and potassium hydroxid is found at the cathode. The chlorin which is first formed reacts with any unacted upon salt of iodin liberating free iodin. When 60 all of the iodin is so liberated, the process may be stopped and the free iodin recovered by any suitable process, such as dissolving in a solvent like carbon tetrachlorid, or carbon disulfid, but the process is preferably 65 continued until all the salts are decomposed. A portion of the chlorin will escape at the anode and may be collected and used for any convenient purpose. The iodin meanwhile is being oxidized, at the loss of a part of the 70 chlorin, to iodic acid. The products derived are potassium hydroxid at the cathode and chlorin and iodic acid at the anode. The iodin may be recovered from the iodic acid by adding ferrous sulfate and sulfuric acid, 75 iron and sulfuric acid, or by any other suitable method.

In practising our other method in treating the ash of seaweeds, we place water in 80 both the anode and cathode compartments of an electrolytic cell, and then add the seaweed ashes to the anode compartment. The ashes are stirred in any convenient manner and the current passed. The soluble salts pass into solution and the changes that occur are the same as disclosed in the previous process, viz: potassium hydroxid being obtained at the cathode and iodin, or chlorin and iodic acid, at the anode. The insoluble residue settles to the bottom of the anode 90 chamber and may be dumped out or separated by any suitable process.

Having thus described our invention we claim as follows:

1. The herein described method for extracting iodin, chlorin, potassium hydroxid and other useful products from the ash of seaweeds, consisting in lixiviating the ash with water, filtering and partially evaporating the solution, subjecting the mother 95 liquor to electrolysis in a cell in which the anode and cathode chambers are separated 100

2

by a diaphragm, thereby oxidizing the liberated iodin to iodic acid, then treating the anode solution with ferrous sulfate and sulfuric acid for separating iodin from such 5 iodic acid.

2. The herein described method for extracting iodin, chlorin, potassium hydroxid and other useful products from the ash of seaweeds, consisting in lixiviating the ash 10 with water, filtering and partially evaporating the solution, subjecting the mother liquor to electrolysis in a cell in which the anode and cathode chambers are separated

by a diaphragm, thereby oxidizing the liberated iodin to iodic acid, then treating the anode solution with iron and sulfuric acid for separating iodin from such iodic acid.

In testimony whereof we affix our signatures in the presence of two subscribed witnesses.

FRANK K. CAMERON.  
RICHARD B. MOORE.

Witnesses:

W. O. ROBINSON,  
HARRY BRYAN.